

# UNITED STATES PATENT OFFICE.

JOSEPH MICHAEL FLANNERY, OF PITTSBURGH, PENNSYLVANIA, ASSIGNOR TO  
STANDARD CHEMICAL COMPANY, OF PITTSBURGH, PENNSYLVANIA.

## HIGH-SPEED STEEL.

1,210,627.

Specification of Letters Patent.

Patented Jan. 2, 1917.

No Drawing.

Application filed September 7, 1916. Serial No. 118,877.

*To all whom it may concern:*

Be it known that I, JOSEPH M. FLANNERY, a citizen of the United States, and a resident of Pittsburgh, in the county of Allegheny and State of Pennsylvania, have invented certain new and useful Improvements in High-Speed Steel; and I do hereby declare the following to be a full, clear, and exact description of the invention, such as 10 will enable others skilled in the art to which it appertains to make and use the same.

This invention relates to improvements in steel alloys, and more particularly to high speed molybdenum steel,—one object of the 15 invention being to produce a high speed steel which shall have added to the qualities of molybdenum thereof, similar qualities derived from the addition of another alloying metal which shall serve to materially reduce the quantity of molybdenum used and at the same time increase the quality of the product in strength, ductility and heat-resisting properties, and enhance its efficiency for use as high speed tool steel.

25 A further object is to produce a high speed molybdenum steel having another metal alloyed therewith which will give superior cutting efficiency to the steel and at the same time permit of a reduction in the 30 amount of molybdenum employed.

With these and other objects in view, the invention consists in a certain novel high speed steel alloy as hereinafter set forth and pointed out in the claims.

35 The invention further consists in molybdenum steel having uranium alloyed therewith.

In the manufacture of my improved high speed steel, I alloy with molybdenum steel, 40 uranium in a proportion appreciably less than that of molybdenum.

It is now common practice in the manufacture of molybdenum steel, to incorporate into a body of steel a comparatively large 45 quantity of molybdenum. This large amount of molybdenum renders the cost of manufacture of molybdenum steel very expensive, and it is the aim of my invention to reduce the cost of such steel by reducing 50 the proportion of molybdenum necessary in its manufacture and at the same time increase the efficiency of the product in all qualities incident to high speed steel.

I have found by incorporating an amount

of uranium from .40 per cent. and not exceeding three per cent. into molybdenum steel containing from three to ten per cent. molybdenum, a high speed steel is produced having all the qualities of molybdenum steel containing a relatively large per cent. 55 of molybdenum, and that the uranium gives to the product greater efficiency, hardness, toughness, thermal absorption, less brittleness, superior cutting quality and replaces a portion of the molybdenum ordinarily employed. An even smaller proportion of 60 uranium than three per cent. may be used with good results.

In the manufacture of my improved high speed steel, I may employ either ferro- 70 uranium or uranium metal, which should be added to the bath of molten steel from five to ten minutes before pouring after de-slagging and after all other alloys have been added. The steel should be poured as soon 75 as the uranium has become melted,—this usually requiring from five to ten minutes unless an electric furnace be employed rather than a crucible when less time will be required for the melting of the uranium.

The presence of uranium in molybdenum steel, not only greatly reduces the proportion of molybdenum necessary, thus reducing the cost of molybdenum content and cost of manufacture of the high speed steel, 85 but it also enhances the hardness, toughness, thermal absorption and general efficiency and durability of the product for the manufacture of cutting tools.

The alloy may be crushed to the desired 90 size and applied to the molten mass while pouring in the ladle, or after the molten mass is in the ladle. It may also be applied in the crucible or furnace.

Having fully described my invention 95 what I claim as new and desire to secure by Letters-Patent, is:—

1. High speed molybdenum steel having uranium alloyed therewith, the uranium replacing a portion of the molybdenum used 100 in ordinary molybdenum steel.

2. High speed steel containing molybdenum and uranium in approximately the relative proportions specified.

3. High speed molybdenum steel having 105 uranium alloyed therewith in proportion less than the proportion of the molybdenum content, the uranium replacing a por-

tion of the molybdenum used in ordinary molybdenum steel.

4. High speed molybdenum steel having uranium alloyed therewith in a proportion as high as three per cent. uranium as a maximum, the uranium replacing a portion of the molybdenum used in ordinary molybdenum steel.

5. High speed molybdenum steel, contain-

ing from three to ten per cent. molybdenum and approximately three per cent. uranium.

In testimony whereof, I have signed this specification in the presence of two subscribing witnesses.

JOSEPH MICHAEL FLANNERY.

Witnesses:

W.M. GANLEY,  
JOSEPH A. KELLY.